

1

3,514,293

**PHOTOGRAPHIC SURFACTANT COMPOSITIONS**  
 William J. Knox, Jr., Rochester, N.Y., assignor to Eastman Kodak Company, Rochester, N.Y., a corporation of New Jersey  
 No Drawing. Continuation-in-part of application Ser. No. 515,179, Dec. 20, 1965. This application Nov. 26, 1968, Ser. No. 779,236  
 Int. Cl. G03c 1/38  
 U.S. Cl. 96—114.5

17 Claims

**ABSTRACT OF THE DISCLOSURE**

This invention relates to compositions which are used in layers of photographic elements or element combinations, said compositions comprising a hydrophilic colloid and an alkylphenoxy poly(hydroxypropylene oxide) having from about 3 to about 15 hydroxypropylene units. In one aspect of this invention, the alkylphenoxy poly(hydroxypropylene oxide) is a compound having the formula:



wherein R represents an alkyl group having from about 6-18 carbon atoms, R' represents a hydrogen atom or an alkyl group having from 1 to 18 carbon atoms and Q represents a polyether group comprising from about 3 to 15 units of hydroxypropylene oxide said polyether group comprising n-propylene and isopropylene moieties. In another aspect, the composition comprises a hydrophilic colloid and the reaction product of an alkylphenol and a glycidol.

This is a continuation-in-part application of Ser. No. 515,179 filed Dec. 20, 1965, and now abandoned.

This invention relates to hydrophilic colloid layers, photographic elements and element combinations containing those layers and to aqueous hydrophilic colloid coating compositions, all of which are characterized by the presence of certain coating aids.

Many image-recording systems use image-forming materials comprising a support such as glass, metal, paper or plastic, overcoated with one or more layers comprising hydrophilic colloidal materials such as gelatin. Silver salt sensitized photographic materials, for example, usually contain one or more aqueous gelatin coatings on film base or paper. The layer containing the silver salt is frequency coated in combination with several other gelatin layers which serve, for example, as carriers for reflective pigments, antihalation dyes or filter dyes, or as undercoatings to improve adhesion, overcoatings to impart abrasion resistance, and the like.

In the coating of such hydrophilic colloid layers, particularly those containing gelatin, it has been customary to employ surface-active agents as coating aids to improve the quality and uniformity of the layers and the ease and reproducibility of their application. The surfactants used often influence other characteristics than the coating per-

2

formance, e.g., surface roughness, permeability to processing solutions, and the like.

Saponin, a material prepared from quillaia bark, has been widely used for this purpose. Being of natural origin, saponin varies in composition according to the source, the method of extracton, and the like, and commercial saponin may include impurities which produce undesirable effects in photographic materials. Saponin has been a reasonably effective coating aid in many applications; however, newer coating procedures which involve increased coating speeds, the application of liquid coating compositions to set (but undried) underlayers and/or the coating of a plurality of layers, have increased the requirements of a satisfactory coating aid and saponin and many other prior art coating aids have been inadequate. Synthetic surfactants have been widely used in recent years in an effort to provide specific requirements in particular coating operations, but a great number of these have been found wanting in one or more particulars when used in recent coating procedures.

ing aids which are photographically inert, but which im-

An object of my invention is to provide new and improved hydrophilic colloid coating compositions;

Another object of my invention is to provide photographic hydrophilic colloid layers containing certain coating aids which are photographically inert, but which impart to said layers good surface characteristics such as a high degree of surface roughness, excellent developer rewettability, lack of repellencies and improved permeability by processing solutions;

A further object of my invention is to provide gelatin-silver halide photographic emulsions containing a certain coating aid which facilitates coating upon a support;

A still further object of my invention is to provide photographic elements containing at least one layer of hydrophilic colloid, for example, gelatin which has excellent characteristics;

Other objects of my invention will appear herein.

I have found that alkylphenoxy poly(hydroxypropylene oxides) can be used very effectively in hydrophilic colloid coating compositions used in making photographic elements. These materials, when incorporated in photographic hydrophilic colloid coating compositions and hydrophilic colloid coatings, increase the ease and efficiency of the coating process and provide a favorably high degree of surface roughness and excellent developer rewettability on coated layers having few or no repellencies, without adversely affecting the photographic properties of the final product. The coating aids of our invention are compatible with both acid- and lime-processed gelatin as well as a wide variety of photographic emulsion addenda such as hardeners, antifoggants, mordants, couplers, antistatic agents and the like.

The alkylphenoxy poly(hydroxypropylene oxides) of this invention are generally of the formula:



wherein R represents an alkyl group having from about 6-18 carbon atoms, preferably from about 8-10 carbon

atoms, and is preferably in the para position; R' represents a hydrogen atom or an alkyl group having from about 1 to 18 carbon atoms and preferably from 6-14 carbon atoms; and Q represents a polyether group comprising from 3 to 15 hydroxypropylene oxide units and preferably consists of at least 8 units which can be interconnected by ether linkages through an oxygen atom on any of the three carbon atoms of the propylene unit, such as to form isopropylene and n-propylene moieties in the group.

The alkylphenoxy poly(hydroxypropylene oxides) can be formed by reacting the alkylphenol with hydroxy compounds according to the procedures normally used to prepare polyglycerol-type compounds. However, the compounds and procedures used in the reaction will, of course, affect the degree of branching and precise structural composition of the product. Since the glycerols, glycerides, glycidols and related compounds required to produce the poly(hydroxypropylene oxide) groups have three possible reaction sites, a high degree of random branching in the molecule is likely to occur, especially when several units are formed in the chain during the reaction as, for example, as when the reaction is continued to form more than 6 units of glycidol. In instances where the alkylphenoxy compound contains upwards of 6 and preferably at least 8 reacted glycidol units, the compound contains sufficient hydroxy and methylol groups to impart improved water solubility and to provide optimum physical and coating characteristics in certain preferred embodiments.

In one preferred embodiment of this invention, an alkylphenoxy polyglycidol is used in coating hydrophilic colloid layers of photographic elements. These compounds are made by reacting the alkylphenol with a glycidol at a temperature above about 100° C. A typical procedure for reacting glycidols is set forth in Belgian Pat. 652,862 granted Sept. 9, 1964.

Typical surface-active agents which are commercially available and which are very useful in my invention include Surfactant 3G (Olin Mathieson Chemical Corp.) which is essentially a para-isonylphenoxy polyglycidol containing an average of 3.3 moles of reacted glycidol; Surfactant 6G (Olin Mathieson Chemical Corp.) which is essentially a para-isonylphenoxy polyglycidol containing an average of above 6 glycidol units; and Surfactant 10G (Olin Mathieson Chemical Corp.) which is essentially a para-isonylphenoxy polyglycidol containing about 10 glycidol units.

The coating aids of this invention are useful in aqueous coating compositions containing hydrophilic colloid. They are useful in coating mixtures of gelatin with other hydrophilic colloid materials which may act, for example, as gel extenders, and to reduce the modulus of elasticity, increase covering power, and the like. Polymers such as copoly(ethyl acrylate-acrylic acid) in monomer ratios of 3:1 to 5:1 and copoly(butyl acrylate-acrylic acid) in monomer ratios of 5:1 to 9:1 are sometimes useful as gelatin extenders. Covering power of emulsions is sometimes increased by incorporating in gelatin-silver halide photographic emulsions such colloids as copolymers of acrylic acid and N-substituted acrylamide as described in French Pat. 1,328,889 and the like.

The utility of surface-active agents in accordance with my invention is not limited to coatings and coating procedures involving photo-sensitive silver halide-gelatin compositions. They can also be used in coating hydrophilic colloid layers which are used in photographic elements or element combinations to be used in conjunction with a photographic element containing a silver halide layer, such as carrier layers for reflective pigments, antihalation dyes, filter dyes, mordants and the like, receiving layers for diffusion transfer, and undercoatings and overcoatings which impart characteristics such as improved adhesion and improved resistance to abrasion. The coating aids denoted as useful in my invention impart to

various hydrophilic colloid layers increased permeability to processing solutions.

It has been further found that the coating aids denoted as useful in my invention can be used in admixture with other surface-active agents such as anionic surfactants, e.g., alkylaryloxyalkylene ether sulfonates, maleopimarates, alkyl sulfates, and amphoteric surface-active agents such as N-alkyl-beta-aminopropionates, acylalkyltaurines, etc.

The coating aids of this invention are also useful in controlling the incidence of longitudinal coating streaks and other defects which occur in the preparation of photographic layers. The reduction of the incidence of coating streaks has been correlated with the increased stainless steel spread values imposed upon hydrophilic colloid solutions by the addition of a coating aid. Stainless steel spread values are obtained by measuring the area over which a sample of a hydrophilic colloid solution will spread on a stainless steel plate. The greater the stainless steel spread values, the more effective is the coating aid in suppressing longitudinal coating streaks. It is shown in the following examples that the coating aids utilized in my invention effectively control the incidence of coating streaks.

The use of coating compositions in accordance with my invention renders the coating of hydrophilic colloid layers in making photographic products adaptable to modern high-speed coating techniques. For example, they operate well in the coating of multilayer photographic elements by the techniques described in British Pats. 855,849 and 929,905, and U.S. Pat. 2,761,791 of Russell.

To illustrate the practice of this invention a number of coatings were prepared by the application to baryta-coated photographic paper base of a silver halide-gelatin photographic emulsion and a clear gelatin overcoat by a multilayer coating technique. The concentration of the surfactant, the developer spread, the coefficient of friction and the number of repellencies per unit area are recorded in the following tables. "Developer Spread" is determined by delivering in a standard manner 1 cc. of developer solution to a surface of photographically sensitized paper carrying a clear gelatin overcoat and measuring the area which develops in a period of 30 seconds. This test indicates how effectively an emulsion will wet. A developer spread of 4.0 cm.<sup>2</sup> or more is desirable.

#### EXAMPLE 1

Coating of emulsion and overcoat layers on paper using, as a coating aid therein, a material of the structure:



wherein Q represents a poly(hydroxypropylene oxide) group containing approximately 10 units of glycidol.

| Surfactant concentration | Repellencies (7.5 ft.²) |                      |                                    |                         |        |      |
|--------------------------|-------------------------|----------------------|------------------------------------|-------------------------|--------|------|
|                          | Wet emulsion, g./lb.    | Wet overcoat, g./lb. | Developer spread, cm. <sup>2</sup> | Coefficient of friction | Bright | Dull |
| 0.0-----                 | 0.5                     |                      | 16.60                              | 0.41                    | None   | None |
| 0.13-----                | 0.5                     |                      | 16.60                              | 0.43                    | None   | None |
| 0.25-----                | 0.5                     |                      | 16.60                              | 0.44                    | None   | None |
| 0.5-----                 | 0.5                     |                      | 16.60                              | 0.42                    | None   | None |
| 0.0-----                 | 0.0                     |                      | 4.90                               | 0.42                    | None   | None |

The following table shows the structures of similar compounds which operate in our invention. In this table x is given as an approximate average value for the number of units of glycidol in the poly(hydroxypropylene oxide) chain represented by Q.

5  
TABLE I

| R                                                    | Position of R | Position of R'                                       | x  |
|------------------------------------------------------|---------------|------------------------------------------------------|----|
| $(\text{CH}_2)_3\text{CC}_2\text{H}_{10}$            | P             | $(\text{CH}_2)_3\text{CC}_2\text{H}_{10}$            | 0  |
| $(\text{CH}_2)_3\text{CCH}_2\text{C}(\text{CH}_3)_2$ | P             | H                                                    | 4  |
| $(\text{CH}_2)_3\text{CCH}_2\text{C}(\text{CH}_3)_2$ | P             | $(\text{CH}_2)_3\text{CCH}_2\text{C}(\text{CH}_3)_2$ | 0  |
| $-\text{C}_{12}\text{H}_{25}$ (iso)                  | P             | H                                                    | 8  |
| $-\text{C}_{14}\text{H}_{31}$                        | m             | H                                                    | 8  |
| $-\text{CH}_3$                                       | P             | $\text{C}_{10}\text{H}_{21}$                         | 6  |
| $\text{C}_5\text{H}_{11}$                            | P             | $-\text{C}_8\text{H}_{17}$                           | 10 |
| $\text{C}_5\text{H}_{11}$                            | P             | $-\text{C}_6\text{H}_{13}$                           | 10 |
| $\text{C}_{10}\text{H}_{21}$                         | P             | H                                                    | 7  |
| $\text{C}_{10}\text{H}_{21}$                         | P             | $-\text{C}_3\text{H}_7$                              | 8  |
| $\text{C}_{13}\text{H}_{37}$                         | P             | $-\text{CH}_3$                                       | 12 |
| $\text{C}_5\text{H}_{11}$                            | P             | $\text{CH}_3\text{CHC}_2\text{H}_3$                  | 7  |
| $\text{CH}_3$                                        | P             | $\text{CH}_3\text{CHC}_{10}\text{H}_{21}$            | 8  |

## EXAMPLE 2

Coating of emulsion and overcoat layers to paper using, as a coating aid, Surfactant 6G sold by Olin Mathieson Chemical Corp.

| Surfactant concentration | Surfactant concentration |                  |                      |                                    |                         |                                      |
|--------------------------|--------------------------|------------------|----------------------|------------------------------------|-------------------------|--------------------------------------|
|                          | Wet emulsion g./lb.      | overcoat, g./lb. | Wet overcoat, g./lb. | Developer spread, cm. <sup>2</sup> | Coefficient of friction | Repellencies (7.5 ft. <sup>2</sup> ) |
| 30                       | 0.0                      | 0.5              | 16.60                | 0.45                               | None                    | None                                 |
|                          | 0.13                     | 0.5              | 16.60                | 0.47                               | None                    | None                                 |
|                          | 0.25                     | 0.5              | 16.60                | 0.47                               | 4                       | 2                                    |
|                          | 0.5                      | 0.5              | 16.60                | 0.50                               | 4                       | 14                                   |
|                          | 0.0                      | 1.0              | 16.60                | 0.49                               | 2                       | 2                                    |
|                          | 0.26                     | 1.0              | 16.60                | 0.49                               | None                    | None                                 |
|                          | 0.5                      | 1.0              | 16.60                | 0.48                               | None                    | None                                 |
| 35                       | 1.0                      | 1.0              | 16.60                | 0.53                               | None                    | None                                 |
|                          | 3.0                      | 2.0              | 16.60                | 0.51                               | None                    | None                                 |
|                          | 0.5                      | 2.0              | 16.60                | 0.53                               | None                    | None                                 |
|                          | 1.0                      | 2.0              | 16.60                | 0.53                               | 1                       | None                                 |
|                          | 2.0                      | 2.0              | 16.60                | 0.49                               | None                    | None                                 |
|                          | 4.0                      | 4.0              | 16.60                | 0.51                               | None                    | None                                 |
|                          | 1.0                      | 4.0              | 16.60                | 0.53                               | 3                       | 2                                    |
|                          | 0.0                      | 4.0              | 16.60                | 0.47                               | None                    | None                                 |
|                          | 2.0                      | 4.0              | 16.60                | 0.50                               | None                    | None                                 |
| 40                       | 4.0                      | 4.0              | 16.60                | 0.47                               | None                    | None                                 |
|                          | 0.0                      | 0.0              | 0.0                  | 0.48                               | None                    | None                                 |
| 40                       | 0.5                      | 16.60            | 0.28                 | None                               | None                    | None                                 |
|                          | 13.90                    | 0.36             | None                 | None                               | None                    | None                                 |
|                          | 16.60                    | 0.37             | 1                    | None                               | None                    | None                                 |
|                          | 16.60                    | 0.39             | 4                    | 4                                  | 4                       | 4                                    |
|                          | 5.31                     | 0.30             | None                 | None                               | None                    | None                                 |

## EXAMPLE 3

Coating of emulsion and overcoat layers to paper using, as a coating aid, Surfactant 6G.

The following examples illustrate the effectiveness of the compounds of my invention when used in combination with other surface-active agents as coating aids.

## EXAMPLE 4

Coating of emulsion and overcoat layers to paper using, as coating aids, mixtures of sodium maleopimarate and Surfactant 10G, sold by Olin Mathieson Chemical Corp., in various proportions by weight.

| Surfactant concentration | Surfactant concentration |                  |                      |                                    |                           |                                      |
|--------------------------|--------------------------|------------------|----------------------|------------------------------------|---------------------------|--------------------------------------|
|                          | Wet emul., g./lb.        | overcoat, g./lb. | Wet overcoat, g./lb. | Developer spread, cm. <sup>2</sup> | Coeffi- cient of friction | Repellencies (7.5 ft. <sup>2</sup> ) |
| 10/0                     | 0.0                      | 0.5              | 4.15                 | 0.48                               | None                      | None                                 |
| 10/0                     | 0.13                     | 0.5              | 4.15                 | 0.52                               | 1                         | 2                                    |
| 10/0                     | 0.25                     | 0.5              | 4.52                 | 0.53                               | None                      | None                                 |
| 10/0                     | 0.5                      | 0.5              | 4.52                 | 0.52                               | None                      | None                                 |
| 0/1                      | 0.0                      | 0.5              | 4.52                 | 0.54                               | None                      | None                                 |
| 9/1                      | 0.13                     | 0.5              | 6.72                 | 0.52                               | None                      | 1                                    |
| 9/1                      | 0.25                     | 0.5              | 6.72                 | 0.51                               | None                      | None                                 |
| 9/1                      | 0.5                      | 0.5              | 10.20                | 0.52                               | None                      | 1                                    |
| 4/1                      | 0.0                      | 0.5              | 5.31                 | 0.54                               | None                      | 1                                    |
| 4/1                      | 0.13                     | 0.5              | 11.90                | 0.54                               | None                      | 1                                    |
| 4/1                      | 0.25                     | 0.5              | 14.50                | 0.52                               | None                      | None                                 |
| 4/1                      | 0.5                      | 0.5              | 16.60                | 0.50                               | None                      | None                                 |
| 7/3                      | 0.0                      | 0.5              | 5.72                 | 0.51                               | None                      | None                                 |
| 7/3                      | 0.13                     | 0.5              | 16.60                | 0.52                               | None                      | None                                 |
| 7/3                      | 0.25                     | 0.5              | 16.60                | 0.52                               | None                      | None                                 |
| 7/3                      | 0.5                      | 0.5              | 16.60                | 0.49                               | None                      | None                                 |
| 1/1                      | 0.0                      | 0.5              | 9.08                 | 0.53                               | None                      | None                                 |
| 1/1                      | 0.13                     | 0.5              | 16.60                | 0.50                               | None                      | None                                 |
| 1/1                      | 0.25                     | 0.5              | 16.60                | 0.52                               | None                      | None                                 |
| 1/1                      | 0.5                      | 0.5              | 16.60                | 0.51                               | None                      | None                                 |
| 3/7                      | 0.0                      | 0.5              | 16.60                | 0.51                               | None                      | None                                 |
| 3/7                      | 0.13                     | 0.5              | 16.60                | 0.49                               | None                      | None                                 |
| 3/7                      | 0.25                     | 0.5              | 16.60                | 0.49                               | None                      | None                                 |
| 3/7                      | 0.5                      | 0.5              | 16.60                | 0.48                               | None                      | None                                 |
| 3/7                      | 0.0                      | 0.0              | 5.31                 | 0.54                               | None                      | None                                 |

**7**  
**EXAMPLE 5**

Coating of emulsion and overcoat layers to paper using, as coating aids, mixtures of Aerosol OT (the dioctyl ester of sodium sulfosuccinic acid, a surface-active agent sold

**8**  
**EXAMPLE 7**

Coating of emulsion and overcoat layers to paper using, as coating aids, mixtures of sodium lauryl sulfate and Surfactant 6G.

| Coating aid                                | Surfactant concentration |                      |                                    | Repellencies (7.5 ft. <sup>2</sup> ) |        |      |
|--------------------------------------------|--------------------------|----------------------|------------------------------------|--------------------------------------|--------|------|
|                                            | Wet emul., g./lb.        | Wet overcoat, g./lb. | Developer spread, cm. <sup>2</sup> | Coefficient of friction              | Bright | Dull |
| Sodium lauryl sulfate/6G ratio by wt. 1/1. | 0.0                      | 0.5                  | 16.60                              | 0.32                                 | None   | None |
|                                            | 0.13                     | 0.5                  | 16.60                              | 0.31                                 | None   | None |
|                                            | 0.25                     | 0.5                  | 16.60                              | 0.34                                 | None   | None |
|                                            | 0.5                      | 0.5                  | 16.60                              | 0.37                                 | None   | None |
|                                            | 0.0                      | 0.0                  | 4.52                               | 0.44                                 | None   | None |

by American Cyanamid Company)<sup>1</sup> and Surfactant 10G in various proportions by weight.

| Ratio by weight of 10G/Aerosol OT | Concentration     |                     | Developer spread, cm. <sup>2</sup> | Coefficient of friction | Repellencies (7.5 ft. <sup>2</sup> ) |      |
|-----------------------------------|-------------------|---------------------|------------------------------------|-------------------------|--------------------------------------|------|
|                                   | Wet emul., g./lb. | Wet overcoat g./lb. |                                    |                         | Bright                               | Dull |
| 10/0                              | 0.0               | 0.5                 | 7.07                               | 0.54                    | None                                 | None |
| 10/0                              | 0.13              | 0.5                 | 16.60                              | 0.53                    | None                                 | None |
| 10/0                              | 0.25              | 0.5                 | 16.60                              | 0.46                    | None                                 | None |
| 10/0                              | 0.5               | 0.5                 | 16.60                              | 0.48                    | None                                 | None |
| 9/1                               | 0.0               | 0.5                 | 16.60                              | 0.48                    | None                                 | None |
| 9/1                               | 0.13              | 0.5                 | 16.60                              | 0.47                    | None                                 | None |
| 9/1                               | 0.25              | 0.5                 | 16.60                              | 0.51                    | None                                 | None |
| 9/1                               | 0.5               | 0.5                 | 16.60                              | 0.46                    | None                                 | None |
| 4/1                               | 0.0               | 0.5                 | 16.60                              | 0.45                    | None                                 | None |
| 4/1                               | 0.13              | 0.5                 | 16.60                              | 0.47                    | None                                 | None |
| 4/1                               | 0.25              | 0.5                 | 16.60                              | 0.49                    | None                                 | None |
| 4/1                               | 0.5               | 0.5                 | 16.60                              | 0.45                    | None                                 | None |
| 7/3                               | 0.0               | 0.5                 | 16.60                              | 0.48                    | None                                 | None |
| 7/3                               | 0.13              | 0.5                 | 16.60                              | 0.46                    | None                                 | None |
| 7/3                               | 0.25              | 0.5                 | 16.60                              | 0.46                    | None                                 | None |
| 7/3                               | 0.5               | 0.5                 | 16.60                              | 0.43                    | None                                 | None |
| 1/1                               | 0.0               | 0.5                 | 9.08                               | 0.42                    | None                                 | None |
| 1/1                               | 0.13              | 0.5                 | 16.60                              | 0.43                    | None                                 | None |
| 1/1                               | 0.25              | 0.5                 | 16.60                              | 0.42                    | None                                 | None |
| 1/1                               | 0.5               | 0.5                 | 16.60                              | 0.40                    | None                                 | None |
| 3/7                               | 0.0               | 0.5                 | 6.16                               | 0.38                    | None                                 | None |
| 3/7                               | 0.13              | 0.5                 | 8.04                               | 0.31                    | None                                 | None |
| 3/7                               | 0.25              | 0.5                 | 16.60                              | 0.35                    | None                                 | None |
| 3/7                               | 0.5               | 0.5                 | 16.60                              | 0.36                    | None                                 | 1    |
| 3/7                               | 0.0               | 0.0                 | 3.80                               | None                    | None                                 | None |

<sup>1</sup> Aerosol OT is bis (2-ethylhexyl) sodium sulfosuccinate and has the structure:



45

**EXAMPLE 8**

Coating of emulsion and overcoat layers to paper using, as coating aids, mixtures of sodium lauryl sulfate and Surfactant 3G.

| Coating aid                                | Surfactant concentration |                      |                                    | Repellencies (7.5 ft. <sup>2</sup> ) |        |      |
|--------------------------------------------|--------------------------|----------------------|------------------------------------|--------------------------------------|--------|------|
|                                            | Wet emul., g./lb.        | Wet overcoat, g./lb. | Developer spread, cm. <sup>2</sup> | Coefficient of friction              | Bright | Dull |
| Sodium lauryl sulfate/3G ratio by wt. 1/1. | 0.0                      | 0.5                  | 16.60                              | 0.36                                 | None   | None |
|                                            | 0.13                     | 0.5                  | 16.60                              | 0.36                                 | None   | None |
|                                            | 0.25                     | 0.5                  | 16.60                              | 0.37                                 | None   | None |
|                                            | 0.5                      | 0.5                  | 16.60                              | 0.38                                 | None   | None |
|                                            | 0.0                      | 0.0                  | 4.52                               | 0.44                                 | None   | None |

**EXAMPLE 6**

Coating of emulsion and overcoat layers to paper using, as coating aids, mixtures of sodium lauryl sulfate (Duponol C sold by DuPont Company) as Surfactant 10G.

| Coating aid                                 | Surfactant concentration |                      |                                    | Repellencies (7.5 ft. <sup>2</sup> ) |        |        |
|---------------------------------------------|--------------------------|----------------------|------------------------------------|--------------------------------------|--------|--------|
|                                             | Wet emul., g./lb.        | Wet overcoat, g./lb. | Developer spread, cm. <sup>2</sup> | Coefficient of friction              | Bright | Dull   |
| Sodium lauryl sulfate/10G ratio by wt. 1/1. | 0.0                      | 0.5                  | 16.60                              | 0.35                                 | None   | Myriad |
|                                             | 0.13                     | 0.5                  | 16.60                              | 0.34                                 | None   | None   |
|                                             | 0.25                     | 0.5                  | 16.60                              | 0.33                                 | None   | None   |
|                                             | 0.5                      | 0.5                  | 16.60                              | 0.33                                 | None   | None   |
|                                             | 0.0                      | 0.0                  | 4.52                               | 0.44                                 | None   | None   |

## EXAMPLE 9

Coating of emulsion and overcoat layers to paper using sodium lauryl sulfate as a coating aid.

| Coating aid           | Surfactant concentration |                      | Developer spread, cm. <sup>2</sup> | Coefficient of friction | Repellencies (7.5 ft. <sup>2</sup> ) |      |
|-----------------------|--------------------------|----------------------|------------------------------------|-------------------------|--------------------------------------|------|
|                       | Wet emul., g./lb.        | Wet overcoat, g./lb. |                                    |                         | Bright                               | Dull |
| Sodium lauryl sulfate | 0.0                      | 0.5                  | 6.16                               | 0.27                    | None                                 | None |
|                       | 0.13                     | 0.5                  |                                    |                         | None                                 | None |
|                       | 0.25                     | 0.5                  |                                    |                         | None                                 | None |
|                       | 0.5                      | 0.5                  |                                    |                         | None                                 | None |
|                       | 0.0                      | 0.0                  |                                    |                         | None                                 | None |

The following examples illustrate the high "stainless steel spread" values obtained for gelatin solutions when a mixture of Surfactant 10G and Aerosol OT is added to the solutions. The "stainless steel spread" values are determined by delivering to a warm stainless steel plate one cubic centimeter of a gelatin solution, cooling the plate to gel the solution and measuring the area over which the solution has spread.

## EXAMPLE 10

Stainless steel spread values for solutions of lime-processed gelatin containing, as coating aids, mixtures, in various ratios by weight, of Surfactant 10G and Aerosol OT.

| Concentration of coating aid in g./lb. of emulsion | Stainless steel spread (cm. <sup>2</sup> ) at various ratios of Surfactant 10G/Aerosol OT |      |      |      |      |       |
|----------------------------------------------------|-------------------------------------------------------------------------------------------|------|------|------|------|-------|
|                                                    | 10/0                                                                                      | 9/1  | 4/1  | 7/3  | 1/1  | 3/7   |
| 0.07                                               | 5.27                                                                                      | 6.13 | 6.93 | 7.20 | 7.27 | 7.5   |
| 0.13                                               | 5.93                                                                                      | 6.73 | 6.67 | 7.83 | 7.97 | 8.0   |
| 0.25                                               | 6.83                                                                                      | 7.53 | 8.63 | 8.69 | 8.90 | 10.10 |
| 0.50                                               | 7.43                                                                                      | 7.97 | 8.93 | 9.04 | 9.10 | 10.47 |

A blank sample of the same gelatin solution tested as above gave a stainless steel spread of 3.8 cm.<sup>2</sup>.

## EXAMPLE 11

Stainless steel spread values for solutions of low-grade, acid-processed pig gelatin containing, as coating aids, mixtures, in various ratios by weight, of Surfactant 10G and Aerosol OT.

| Concentration of coating aid in g./lb. of emulsion | Stainless steel spread (cm. <sup>2</sup> ) at various ratios of surfactant 10G/aerosol OT |      |      |      |      |      |
|----------------------------------------------------|-------------------------------------------------------------------------------------------|------|------|------|------|------|
|                                                    | 10/0                                                                                      | 9/1  | 4/1  | 7/3  | 1/1  | 3/7  |
| 0.7                                                | 5.90                                                                                      | 5.29 | 6.87 | 6.60 | 6.87 | 7.33 |
| 0.13                                               | 6.30                                                                                      | 6.20 | 7.10 | 7.50 | 7.50 | 7.40 |
| 0.25                                               | 6.57                                                                                      | 7.17 | 7.23 | 7.77 | 7.80 | 8.20 |
| 0.50                                               | 6.77                                                                                      | 7.47 | 7.70 | 8.37 | 8.43 | 8.73 |

A blank sample of the same gelatin solution tested as above gave a stainless steel spread of 3.9 cm.<sup>2</sup>.

The coating aids of this invention can be used with any of the conventional hydrophilic water-permeable binding materials employed in the preparation of photographic silver halide emulsions and elements, as exemplified by gelatin, colloidal albumin, cellulose derivatives, synthetic resins such as polyvinyl compounds, e.g., acrylamide polymers and the like, as well as mixtures of these materials.

The coating aids of this invention can be used to coat hydrophilic colloids on a wide variety of supports. The hydrophilic colloid layers can be coated on one or both sides of the support, if desired. Typical supports are cellulose nitrate film, cellulose ester film, polyvinyl acetal film, polystyrene film, polyethylene terephthalate film, and related films or resinous materials, as well as glass, paper, metal and the like. Supports such as paper, which are coated with alpha-olefin polymers, particularly polymers of alpha-olefins containing two or more carbon atoms, as exemplified by polyethylene, polypropylene, ethylene-butene copolymers and the like, can also be employed.

The coating aids employed in the practice of this invention can be used in various kinds of silver halide photographic emulsions. In addition to being useful in

ortho-chromatic, panchromatic and infrared-sensitive emulsions, they are also useful in X-ray and other non-optically sensitized emulsions. They can be used in sulfur and gold sensitized silver halide emulsions. Emulsions containing various types of silver salts can be used such as silver bromide, silver iodide, silver chloride or mixed silver halides such as silver chlorobromide, silver bromo-iodide or silver chloro-iodide. The coating aids employed in the practice of this invention can be used to coat hydrophilic colloid layers in elements intended for color photography, for example, silver halide emulsions containing color-forming couplers or emulsions to be developed in solutions containing couplers or other color-generating materials.

The coating aids of the invention can be employed to coat hydrophilic colloid layers containing mordants, pigments, such as titanium dioxide, zinc oxide, silica particles, manganese dioxide, absorbing dyes and the like.

Photographic layers coated according to this invention can be used in diffusion transfer processes which utilize a non-developed silver halide in the non-developed silver halide in the non-image areas of the negative to form a positive by dissolving the undeveloped silver halide and precipitating it on a receiving layer in close proximity to the original silver halide emulsion layer. Such processes are described in Rott, U.S. Pat. 2,352,014, Land, U.S. Pat. 2,543,181, and Yackel et al., U.S. Pat. 3,020,155. The silver halide emulsions described herein can also be used in color transfer processes which utilize the diffusion transfer of an imagewise distribution of developer, coupler or dye from a light-sensitive layer to a second layer while the two layers are in close proximity to one another. Color transfer processes of this type are described in Yutzy, U.S. Pat. 2,856,142; Land et al., U.S. Pat. 2,983,606, Whitmore et al., British Pats. 904,364 and 840,731; and Whitmore et al., U.S. application Ser. No. 392,471.

The invention has been described in considerable detail with particular reference to certain preferred embodiments thereof, but it will be understood that variations and modifications can be effected within the spirit and scope of the invention as described hereinabove and in the appended claims.

I claim:

1. An aqueous coating composition comprising an aqueous dispersion of a hydrophilic colloid and a silver halide containing therein a compound having the formula:



wherein R represents an alkyl group having from about 6-18 carbon atoms, R' represents a hydrogen atom or an alkyl group having from 1 to 18 carbon atoms and Q represents a polyether group comprising from about 3 to 15 units of hydroxypropylene oxide said polyether group comprising n-propylene and isopropylene moieties.

2. The composition according to claim 1 wherein said R is an isonylon group in the para position of said phenoxy.

## 11

3. The composition according to claim 1 wherein Q consists of at least 8 hydroxypropylene units.

4. The composition according to claim 1 wherein R' is a hydrogen atom.

5. The composition according to claim 1 wherein said hydrophilic colloid is a gelatin.

6. An aqueous coating composition comprising an aqueous dispersion of a hydrophilic colloid and a silver halide containing therein an alkylphenoxy poly(hydroxypropylene oxide) having a polyether group from about 3 to 15 hydroxypropylene oxide units said polyether group comprising n-propylene and isopropylene moieties and the said alkyl of the alkyl-phenoxy group contains at least 6 carbon atoms.

7. A composition according to claim 6 wherein said alkylphenoxy poly(hydroxypropylene oxide) is prepared by reacting an alkylphenol with glycidol.

8. A composition according to claim 7 wherein said alkylphenoxy polyglycidol contains at least 8 units of reacted glycidol.

9. A composition according to claim 6 containing an anionic surface-active agent in combination with said alkylphenoxy poly(hydroxypropylene oxide).

10. A composition according to claim 6 wherein said anionic surface-active agent is sodium maleopimarate.

11. A composition according to claim 9 wherein said anionic surface-active agent is sodium lauryl sulfate.

12. A composition according to claim 9 wherein said anionic surface-active agent is bis(2-ethylhexyl)sodium sulfosuccinate.

13. A photographic element combination comprising (1) a support, (2) at least one layer containing a silver halide and (3) at least one layer containing a hydrophilic colloid and a compound having the formula:



## 12

wherein R represents an alkyl group having from 6 to 18 carbon atoms, R' represents a hydrogen atom or an alkyl group having 1 to 18 carbon atoms and Q represents a polyether group comprising from 3 to about 15 units of hydroxypropylene oxide, said polyether group comprising n-propylene and isopropylene moieties.

14. A photographic element combination according to claim 13 wherein said alkylphenoxy poly(hydroxypropylene oxide) is prepared by reacting an alkylphenol with glycidol.

15. A photographic element combination according to claim 14 wherein said alkylphenoxy polyglycidol consists of an alkylphenol reacted with at least 8 units of a glycidol.

16. A photographic element combination according to claim 13 wherein said hydrophilic colloid is a gelatin.

17. A photographic element according to claim 13 wherein said silver halide-containing layer and said alkylphenoxy poly(hydroxypropylene oxide) - containing layer are coated on the same support.

20

## References Cited

## UNITED STATES PATENTS

|           |         |                         |          |
|-----------|---------|-------------------------|----------|
| 2,089,569 | 8/1937  | Orthner et al. -----    | 260—106  |
| 2,213,477 | 9/1940  | Steindorff et al. ----- | 260—613  |
| 2,752,246 | 6/1956  | Weaver -----            | 96—114   |
| 3,201,252 | 8/1965  | Knox et al. -----       | 96—114.5 |
| 3,415,649 | 12/1968 | Nishio et al. -----     | 96—114.5 |

## FOREIGN PATENTS

|    |         |        |          |
|----|---------|--------|----------|
| 30 | 652,862 | 9/1964 | Belgium. |
|----|---------|--------|----------|

NORMAN G. TORCHIN, Primary Examiner

M. F. KELLEY, Assistant Examiner

35

UNITED STATES PATENT OFFICE  
CERTIFICATE OF CORRECTION

Patent No. 3,514,293 Dated May 26, 1970

Inventor(s) William J. Knox, Jr.

It is certified that error appears in the above-identified patent and that said Letters Patent are hereby corrected as shown below:

In Column 1, line 52 (page 1, line 11 of application), "frequency" should read ---frequently---.

In Column 2, line 21, delete entire line.

In Column 2, line 24, (page 2, line 10 of application), "nvention" should read ---invention---.

In Column 4, line 36, (page 6, line 18 of application), "concentration" should read ---concentrations---.

In Column 9, line 37, (page 13, line 12 of application), "testsd" should read ---tested---.

Claim 10, line 1 (Claim 10 of application), "Claim 6" should read ---Claim 9---.

Signed and sealed this 29th day of February 1972.

(SEAL)

Attest:

EDWARD M.FLETCHER, JR.  
Attesting Officer

ROBERT GOTTSCHALK  
Commissioner of Patents